

Dec. 4, 1962

962 A. M. LEAS 3,067,126  
PRODUCTION OF HIGH TEMPERATURE, HIGH PERFORMANCE, AND  
HIGH ENERGY HYDROCARBON FUELS  
Filed Aug. 6, 1959

Filed Aug. 6, 1959



## 1

3,067,126

## PRODUCTION OF HIGH TEMPERATURE, HIGH PERFORMANCE, AND HIGH ENERGY HYDRO-CARBON FUELS

Arnold M. Leas, 803 Bellefonte Princess Road,  
Ashland, Ky.Filed Aug. 6, 1959, Ser. No. 833,664  
10 Claims. (Cl. 208—66)

This invention relates to a process for producing improved high temperature, high performance, and high energy hydrocarbon fuels for turbojet, ramjet, and rocket engines. More specifically, it is concerned with making readily available large quantities of a wide variety of improved hydrocarbon fuels at relatively low cost.

This application is a continuation-in-part of my prior application Serial No. 762,432, filed September 22, 1958, now abandoned.

The need for improved hydrocarbon fuels for aircraft is evident upon consideration of their increased speed, increased range, and flight at higher altitudes. For an aircraft to fly at increased speed, the hydrocarbon fuel must display increased thermal stability, greater reactivity, and improved combustion properties. For an aircraft to go farther, the hydrocarbon fuel must possess higher combustion efficiencies under more stringent conditions together with greater heat content per unit weight and/or per unit volume. For an aircraft to go higher, the hydrocarbon fuel must burn at lower pressure and must have higher reactivity and lower vapor pressure to prevent premature vaporization.

An object of this invention is the production of a high performance hydrocarbon fuel which possesses improved thermal stability. Thermal stability is defined as the resistance of a fuel to decomposition at elevated temperatures. Such decomposition results in the formation of undesirable deposits in the fuel system and causes excessive vapor pressures. Obtaining better thermal stability is the greatest problem facing aircraft propulsion today. At the operating temperatures concomitant higher propulsion speeds, the thermal stability of high performance hydrocarbon fuels becomes critically important.

Another object of this invention is the provision of a high energy hydrocarbon fuel with low vapor pressure, which retains good flow characteristics at the very low temperatures encountered at high altitudes, in order to maintain desirable handling characteristics and component performance and to prevent center of gravity surge problems.

A more specific objective of this invention is the production of an alkylated naphthenic hydrocarbon of higher heat content than conventional jet fuels. In the performance of liquid-fuel rockets, such a compound has been found to possess desirable characteristics in comparison with the liquid boranes, the low density of which offsets the theoretical increase in specific impulse.

A further objective of this invention is the production of alkylated naphthenic hydrocarbon that is more resistant to nuclear radiation than conventional jet fuels heretofore available. The alkylated synthetic naphthenic hydrocarbons of this invention display much greater resistance to gamma radiation than conventional jet fuels.

A still further objective of the invention is the provision of a process wherein various aromatic feedstocks of different boiling points and heat contents, e.g. single rings (benzene), condensed rings (naphthalene or tetralin), isolated rings (biphenyl), along with olefinic gases, may be charged to yield products of specific distillation range as required for the many weapon systems which travel at varying speeds. In order to make many different types of hydrocarbon fuels economically, a producer

## 2

needs an extremely flexible process to meet the urgent and rapidly changing demands of the military and civilian industries. An example of the flexibility of this process is that its operating conditions can be changed in order to alkylate one or more sidechains to the aromatic rings in order to control the distillation range of the end product.

Another objective of this invention is the provision of a chemically pure product. This is effected by simple distillation whereby the reacted products which have a higher boiling point than the charge stock are removed as essentially pure aromatics. The heavy aromatic product may be removed hot from the distillation tower bottoms and fed into the hydrogenation unit to produce a pure end product.

15 A specific objective of this invention is the production of hydrocarbon fuels which will pass both the Standard CRC Coker test and the Research CRC Coker test. These are tests which have been adopted to evaluate the performance characteristics of fuels by subjecting them to 20 conditions generally simulating the adverse conditions which may exist in use.

The Standard CRC Coker test consists of pumping the fuel at ambient temperature over an aluminum preheater tube into a second heater and thence into a standardized filter. The effluent from the filter is water-cooled and passed into a receiver. The pressure drop through the filter furnishes a measure of the quantity of the products of thermal decomposition of the fuel retained by the filter, and hence is a measure of the fuel's stability under heat. 25 Deposits on the heat exchanger or pre-heater tube are also compared against standards to establish a so-called pre-heater rating. The Standard CRC Coker operates over a range of operating conditions as follows:

Pumping flow rate, lbs./hr. 2-8.  
35 Preheater temperature. Ambient—500° F.  
Filter temperature, ° F. 400-600.  
Pumping pressure, p.s.i.g. 150.  
Duration of run, hrs. 5-15.  
No preheating chamber prior to run.

40 The Research CRC Coker test is designed for the testing of advanced hydrocarbon high performance fuels. It consists of pumping the fuel from a heated stainless steel reservoir, which can be varied from ambient to 300 F. temperature, to an aluminum or stainless steel pre-heater tube into a second heater and thence into a filter. The effluent from the filter is water-cooled and passed into 45 a receiver. The operating conditions of the Research CRC Coker may be varied over a range as follows:

50 Pumping flow rate, lbs./hr. 2-10.  
Preheater temperature. Ambient—800° F.  
Filter temperature, ° F. 500-900.  
Pumping pressure, p.s.i.g. 250.  
Duration of run, hrs. 5-15.

55 The heating reservoir is equipped with a mixer and can be blanketed with air and/or inert gas in order to assimilate wing storage conditions.

60 The development of high performance hydrocarbon fuels has become necessary because all of the present conventional hydrocarbon fuels fail to pass the Research Coker test. This invention permits producers to make high performance hydrocarbon fuels that will pass the Research Coker test and also flight tests. For example, the Research and Standard CRC Coker preheater ratings 65 range from 0 (best) to 8 (worst), and the filter ratings range from 0 (best) to 25 inches (worst). Fuels may be produced according to this invention which will pass the Research CRC Coker test with a preheater rating of 70 3 maximum and a filter pressure drop of 1.0 inch maximum.

A further object of this invention is the provision of a

simple and economical process for producing from inexpensive petroleum charge stocks high temperature, high performance, and high energy hydrocarbon fuels which are more resistant to nuclear radiation, which process, because of the mild operating conditions utilized, is adapted to be practiced with relatively simple and inexpensive equipment. The process facilities can, in fact, be made readily available by a simple conversion of conventional petroleum refinery facilities.

The process of this invention consists principally in the reaction of a catalytic reformate which contains benzene, toluene, and heavier aromatics boiling in the range from 150° to 450° F., with a light olefinic hydrocarbon which is preferably ethylene, propylene, and butylene, or a mixture thereof, using phosphoric acid catalyst, solid or liquid, in the presence of hydrogen to effect reaction at moderate temperature, for example, 150°-450° F., and at moderate pressure, for example 150-300 p.s.i.g. to produce an essentially pure high boiling aromatic hydrocarbon, and then hydrogenating the high boiling aromatic compounds to form a naphthenic end product. A further aspect of the invention is a novel treatment of this naphthenic product with hot and cold clay to improve the thermal stability of the end product, as subsequently described.

The reaction preferably is conducted in the presence of hydrogen, some of which may be recycled to the reaction zone in order to minimize carbon deposition and to improve catalyst activity. It has been discovered that the presence of hydrogen at the site of the reaction, obtained by injection of hydrogen if necessary, contributes very advantageously to the maintenance of high catalyst activity and catalyst life, particularly in the charging of heavier feed stock, and also reduces carbon deposition and suppresses undesirable side reactions.

In order to maintain proper hydration of the phosphoric acid catalyst, water, alcohol, or another suitable source of hydroxyl groups may be added to the alkylation zone. The mild operating conditions are made practical by operating at low space velocity. The low operating temperature and pressure enable the use of standard carbon-steel equipment which is readily available in most petroleum refineries.

The low boiling hydrocarbons or unreacted components may be recycled to obtain high yields of essentially pure high boiling aromatics. These are separated by simple fractionation and constitute a charging stock for a second step wherein the high boiling aromatics are hydrogenated by means of a suitable hydrogenation catalyst, e.g., platinum or nickel, under mild operating conditions (300°-600° F. and 300-1000 p.s.i.g.).

A novel feature of this invention resides in the discovery that the phosphoric acid catalyst functions to promote the alkylation of aromatic by olefinic components present at the site of reaction and simultaneously promotes dehydrogenation in the conversion of paraffin components to olefins which then alkylate the aromatics and/or cyclize olefins to additional aromatics which further alkylate. From present evidence it appears feasible under various plant operating conditions to recycle all of the low boiling hydrocarbons to the alkylating dehydrocyclization catalyst to permit almost complete conversion of the charge stock to high boiling aromatics suitable for hydrogenation to the desired product. However, for given plant facilities, increased quantities of the desired high energy fuel product can be obtained by diverting a portion of the recycle stock for use as valuable by-product material suitable for gasoline blending or as petrochemical charge stock. Material balances indicate that sufficient dehydrogenation occurs in the alkylation step to provide a portion of the hydrogen required to saturate the heavy aromatics in the second or hydrogenation step of the process. Up to approximately 25% motor alkylate and/or iso-octane economically may be included in the reformate charge to provide iso-octyl benzene which can

also be subsequently saturated with hydrogen to increase the heating value of the finished product.

The process of this invention also includes incorporating biphenyl and other polycyclic hydrocarbons which can be alkylated with ethylene and/or propylene and/or butylene to produce products which can be further hydrogenated to increase the heating value and density of the finished product. Thus, products of this invention are essentially pure alkyl naphthenic hydrocarbons, principally dimeric and trimeric, which have unusually good thermal stability properties, combined with high energy content. The process possesses sufficient flexibility to enable special end products to be obtained by variations in the feed stock in order to satisfy specific or specialty requirements.

The following examples are given to indicate results obtainable by the use of the present process, although they are not intended to limit the scope of the invention to exact correspondence herewith.

#### EXAMPLE 1

A liquid charge consisting of 75% by liquid volume of catalytic reformate (boiling point 140°-250° F.) and 25% heat cut alkylate (boiling point 140°-250° F.) with sufficient propylene is charged to the phosphoric acid catalyst reactor to produce a product which on fractionation yields 35% heavy aromatics (boiling point approximately 375°-600° F.) and 65% of a product boiling below 375° F. which may be diverted or recycled; if recycled, this fraction on the second and third pass yields comparable quantities of the 375° F. residue without impairing the desirable properties of the fraction. When the 375° F. residue heavy aromatic fraction is saturated with hydrogen, it yields a product having an API gravity of about 40°, boiling range of 375°-600° F., freezing point of below -90° F., viscosity at -30° F. of 20 centistokes, net heating value of 18,700 B.t.u./lb. or 128,282 B.t.u./gal., and a CRC Research Coker rating of substantially less than 1 inch Hg filter pressure drop and a maximum preheater rating of No. 2 under the following conditions:

|                             | Example 1<br>Fuel | Current Con-<br>ventional<br>Jet Fuel |
|-----------------------------|-------------------|---------------------------------------|
| Pumping Flow Rate, lbs./hr. | 6                 | 6                                     |
| Preheater Temperature, ° F. | 500               | 500                                   |
| Filter Temperature, ° F.    | 600               | 600                                   |
| Pumping Pressure, p.s.i.g.  | 250               | 250                                   |
| Duration of Run, hrs.       | 5                 | 5                                     |
| Results of Test:            |                   |                                       |
| Hg ΔP, inch                 | 0.03              | 18                                    |
| Preheater Tube (Al) Deposit | 2                 | 8                                     |
| Final Rating                | Passing           | Not Passing                           |

Pre-test treatment consisted of heating and agitating the fuel in the presence of air at 300° F. for 5 hours. From the foregoing data, it will be seen that the present invention provides a process for manufacturing high performance hydrocarbon fuels capable of passing the Research CRC Coker Test, which conventional jet fuels completely fail.

According to the Standard CRC Coker test procedure previously identified, air is not present during test pre-heating or thereafter. However, air is present in wing tanks of aircraft during high speed flight, and skin friction causes appreciable rise in the temperature of the fuel therein, which may continue over prolonged flight periods. The best high energy hydrocarbon fuels presently available, when exposed to heat and air under such conditions, give Research CRC Coker ratings which are considerably less desirable than the coker ratings furnished by the same fuels not subjected to the heat and air environment. In contrast, fuels prepared in accordance with the present invention display the same Research CRC Coker rating whether preheated according to the test in the absence of air or preliminarily exposed

75

5

to air at a temperature of 300° F. for 5 hours prior to preheating and testing according to the standard procedure. This shows the remarkable thermal stability of the fuels under conditions which are even more adverse than those in the Standard CRC Coker procedure.

#### EXAMPLE 2

Using the same charge stock as in Example 1 plus 10% by weight of biphenyl added thereto, a finished fuel product is produced having similar properties and Research CRC Coker rating to those shown in Example 1 with the exception that the API gravity is 35° and the net heating value is increased to 18,750 B.t.u./lb. and 132,675 B.t.u./gal.

#### EXAMPLE 3

A liquid charge consisting of catalytic reformate (boiling point 140°-250° F.) with sufficient propylene is charged to the phosphoric acid catalyst reaction to produce a product which on fractionation yields 23% heavy aromatics (boiling point 375°-600° F.) and 77% of a product boiling below 375° F. which may be diverted or recycled; if recycled, this fraction on the second and third pass yields comparable quantities of the 375° F. residue without impairing the desirable properties of the fraction. When the 375° F. residue heavy aromatic fraction is saturated with hydrogen, it yields a product having an API gravity of about 40°, boiling range of 375°-600° F., freezing point of below -90° F., viscosity at -30° F. of 20 centistokes, net heating value of 18,650 B.t.u./lb. or 128,125 B.t.u./gal., and a Research CRC Coker rating similar to that of Example 1.

#### EXAMPLE 4

A liquid charge consisting of heavy catalytic reformate (boiling point 250°-450° F.) with sufficient propylene is charged to the phosphoric acid catalyst reactor in the presence of hydrogen to produce a product which on fractionation yields 65% high purity aromatics (boiling point approximately 415°-650° F.) and 35% of a product boiling below 415° F. which may be diverted or recycled; if recycled, this fraction on the second and third pass yields comparable quantities of the 415° F. residue without impairing the desirable properties of the fraction. When the 415° F. residue heavy aromatic fraction is saturated with hydrogen, it yields a product having an API gravity of about 31.5°, boiling range of 390°-625° F., freezing point of below -100° F., viscosity at -30° F. of 14.5 centistokes, net heating value of 18,420 B.t.u./lb. or 133,140 B.t.u./gal., and a similar Research CRC Coker rating as shown in Example 1. The product from this charge stock is primarily a mixture of alkylated monocyclic and alkylated bicyclic naphthenes.

#### EXAMPLE 5

The pure heavy aromatic hydrocarbon from the reactor unit as illustrated in Example 1 can be blended with naphthalene and then charged to the hydrogenation unit to make a product that is similar to the finished product shown in Example 4. Likewise tetralin can replace the naphthalene as charge to the hydrogenation unit along with the pure heavy aromatic in Example 1 to make a product similar to that in Example 4.

#### EXAMPLE 6

Following is an example of the improvement in thermal stability which is conferred upon a fuel product by hot and cold clay treatment following hydrogenation.

Naphthalene and/or tetralin can be charged directly to the hydrogenation unit to produce high quality decalin with an API gravity of about 30.1°, boiling range of 350°-390° F., freezing point of -40° F., viscosity at -30° F. of 11.6 centistokes, net heating value of 18,412

6

B.t.u./lb. or 134,242 B.t.u./gal., and a Research CRC Coker rating as shown below.

|   |                             |     |
|---|-----------------------------|-----|
| 5 | Pumping flow rate, lbs./hr. | 6   |
|   | Preheater temperature, ° F. | 550 |
| 5 | Filter temperature, ° F.    | 650 |
|   | Pumping pressure, p.s.i.g.  | 250 |
|   | Duration of run, hrs.       | 5   |

Pretest treatment consists of heating and agitating in 10 the presence of air at 300° F. for 5 hours.

#### Results

|    | Hot and Cold Clay Treatment      |         |
|----|----------------------------------|---------|
|    | Before                           | After   |
| 15 |                                  |         |
|    | Hg AP, inch.....                 | 22      |
| 20 | Preheater Tube (Al) Deposit..... | 7       |
|    | Final Rating.....                | 2       |
|    | Not Passing                      | Passing |

Decalin is limited in its application because of its high 25 volatility, relatively high freeze point, and high price. The distillation range of decalin is 360°-390° F. whereas many of the higher speed weapon systems require hydrocarbon fuels that have a distillation range between 375°-600° F. such as illustrated in Examples 1 through 5. Likewise the price of decalin is approximately ten times 30 the cost of products described in Examples 1 and 3. The availability of decalin is very limited compared to the products described in Examples 1 through 5.

In aircraft armed with nuclear projectiles the fuel for 35 the aircraft inevitably is or will be subjected to gamma radiation. Such radiation has been found to exert serious decomposing effects upon various hydrocarbons and in particular upon JP-4, JP-5, and JP-6 fuels which constitute the fuels now commonly used in such aircraft. The adverse effect of radiation is indicated by decrease 40 of Research CRC Coker rating of the fuel. However, exposure to gamma radiation of the fuels in the present invention has been found to have no significant effect upon their coker rating.

One method suitable for the practice of the process of 45 this invention is illustrated schematically in the accompanying drawing. Olefins from a charge component comprising ethylene, butylene, and propylene or mixtures thereof, proportioned in relation to the end product desired, plus whatever inert gases such as pentane, butane, 50 ethane, and propane that may be present therein, enter the system through line 1. Where these gases are supplied from cracking processes, hydrogen also normally will be present; if not, hydrogen as required in the practice of the process is supplied as later described. The 55 gases entering the system through line 1 are first prepared for use by treating them to remove hydrogen sulfide and ammonia as is indicated generally at 2. This type of gas purification is conventional and therefore is not described here in detail.

60 From the preparation step 2 the gases are delivered by a compressor 3 to gas charge line 4 which is valved as at 5. A portion of the compressor discharge is preferably passed through line 6 into an absorber 7.

The paraffinic liquid feed components, i.e., C<sub>6</sub> catalytic 65 reformate and such alkylate as iso-octane which it is desired to employ, enter the system through line 8 and pass into a depentanizer 9 through which entrained pentane is removed from the charge and discharged through line 10. The balance of the liquid charge passes through 70 line 11 to a splitting tower 12 which is operated to separate heavy or high boiling reformate and alkylate from the desired lighter fractions of these components. The heavy product is discharged from the system through line 13 and passes to storage for use as a gasoline blending additive or for other desired uses, while the light 75

reformate and alkylate enter the reaction system through a pump 14 which discharges into feed line 15. However, a portion of the liquid feed is diverted through the line 16 into the absorber 7 wherein it absorbs components of the gas feed and rich oil from the absorber, re-enters the feed stream through line 17, the flow rate through the absorber being adjusted by means of valve 18. Feed gases which are insoluble in the absorber liquid, such as methane and nitrogen, are ejected from the system through line 19. Some excess hydrogen is lost in this procedure, but a typical refinery gas contains hydrogen substantially in excess of the amount required in the practice of the present process, so this loss is of no immediate consequence.

The combined liquid and gas charge in line 15 now passes through a heater 20 and then into reactor 21.

In the system illustrated, the reactor contains a fixed bed of phosphoric acid as a catalyst. In the preferred operation the phosphoric acid is of 60-70% strength and is disposed upon a carrier such as silicon dioxide or kieselguhr. The water content of the catalyst preferably is approximately 12-15%; for convenience, the catalyst may be represented typically as  $\text{SiO}_2 \cdot \text{P}_2\text{O}_5 \cdot \text{H}_2\text{O}$ . Loss of water from the catalyst as the reaction proceeds is made up by addition of water or alcohol introduced suitably into the line 15. The use of alcohol in place of water generally permits better control of the OH addition rate.

Within the reactor a number of different reactions take place as is subsequently discussed. Some of these are exothermic and some endothermic, by reason of which it is generally unnecessary to provide for substantial removal of heat from the reactor. If necessary, temperature reduction readily may be obtained through quenching effect by diverting the feed stream through the heater 20 or by addition of a recycle stream as is discussed at a later point in the specification.

When the gas charge is deficient in hydrogen, hydrogen may be supplied directly to the reactor 21 as indicated by the dotted line 22.

Mixed products of the reaction leave the reactor through line 23 and pass to a first fractionator 24 wherein light aromatic hydrocarbons such as ethyl benzene are removed. The bottoms product of this fractionator is passed through line 25 to a second fractionator 26 wherein heavier aromatic hydrocarbons such as cumene are removed. The bottoms product of the second fractionator, as flowing in line 35, now constitutes an essentially pure aromatic hydrocarbon which, under the preferred temperature of the second fractionator, boils at a temperature of approximately 375°-600° F.

Each of the fractionators 24 and 26 preferably is equipped for reflux operation. Thus, in unit 24, the overhead product passes from line 27 through a condenser 28 to a receiver 29 from which the reflux is returned to the fractionating column through line 30. Gas liberated from the overhead fraction is discharged from the receiver through line 31 as a fuel gas. The reflux system in the second fractionator 26 is the same, but in this case no vent gas line is required since non-condensable gases are stripped from the product in the first fractionating operation.

In the practice of the process the low boiling and high boiling aromatic hydrocarbons removed at fractionators 24 and 26 either may be used as petrochemical feed stocks or may be used for blending with gasoline. However, an important economic advantage in the practice of the present invention is provided by the utilization of these fractions as recycle charge stock to the reactor. For this purpose the components as withdrawn from the fractionators through lines 32 and 33 may be mixed and recycled to the reactor 21 through line 34. This recycle stream provides convenient means for controlling the temperature in the reactor if necessary.

In the second phase of the production of thermally stable, high energy liquid fuels according to the present invention, the aromatic hydrocarbons flowing in line 35 are hydrogenated for conversion of the aromatic hydrocarbons to naphthenes. This operation is conducted at the hydrogenator 37. The charge, before entering the hydrogenator, passes through a heater 36 through which the temperature may be controlled. Hydrogenation is conducted in the presence of a suitable hydrogenation catalyst such as platinum or nickel on a suitable carrier such as aluminum oxide. For hydrogen supply to the hydrogenator, reformer off-gas may be used, in which event the gas is treated to effect removal of hydrogen sulfide by conventional means as indicated generally at 39.

The naphthene stream, discharged from hydrogenator 37 in line 42, passes through a condenser 43 into a liquid gas separator 44. Hydrogen gas liberated at the separator 44 is recycled by means of a compressor 41 and return line 40 while the hydrogenated liquid product is passed from the receiver 44 through a line 45 into a stripper 46 where residual hydrogen or inert gases are removed. These are discharged through line 47, and the end product is discharged through line 48.

Next the liquid product discharged from stripper 46 is preferably subjected to a hot clay treatment followed by a cold clay treatment. This treatment has been found effective to remove small traces of undesirable organometallic compounds containing copper, lead, and arsenic which otherwise adversely affect heat stability. In addition, however, it has been discovered that even small amounts of olefinic compounds present in fuel impair its Coker Rating, and that the hot clay treatment followed by cold clay treatment is effective to improve the Coker rating, apparently by effecting the removal of such compounds. Such improvement is indicated, typically, in the data accompanying Example 6. Thus, the liquid product from the stripper 46 is discharged through line 48 to a hot clay reactor 49 which is charged with a suitable clay such as bauxite and which is operated at a temperature of approximately 300°-650° F., preferably 600° F. Flow rate is adjusted to a space velocity of approximately one, which allows ample time of residence to permit polymerization of unstable hydrocarbons such as mono- and diolefins to occur. From the hot clay reactor the liquid product is discharged through line 50 and through a cooler 51 to a cold clay tower 52 similarly charged with a suitable clay such as bauxite. The cold clay treatment is effective to filter the polymerized hydrocarbons and metal compounds from the stream. The end product is discharged from the system through line 54 to storage. This finished end product is the high temperature fuel possessing high thermal stability, resistance to radiation, high performance properties, together with higher energy than other presently known hydrocarbon fuels.

As previously noted, the invention is practiced at relatively nominal temperature and pressure conditions, which permits carbon steel vessels and piping to be used at low cost. In the reactor the preferred temperature of operation is approximately 300°-400° F. and the pressure approximately 200-400 p.s.i.g. The low cost of the carbon steel construction permits a reactor to be employed which is sufficiently large to enable a low space/hourly rate velocity to be maintained. For example, in the physical operation the space/hourly rate velocity may be .05 to 1.0, and preferably approximately 0.1 (gallons combined feed per hour per pound of catalyst).

It will be understood that the proportion of gas feed to liquid feed as well as the chemical constitution of each will affect the properties of the end product. In general, the proportions preferably are adjusted so that 2 to 3 mols of ethylene, propylene, or butylene, or mixtures

thereof, are available for each mol of benzene in the liquid feed, and hydrogen is maintained in quantity to furnish approximately one-half mol of hydrogen per mol of benzene in the liquid feed. Saturation of the aromatic hydrocarbons at the hydrogenator 37 preferably is conducted at a temperature of approximately 450° F.

To effect removal of light aromatic hydrocarbons, the first fractionator may be operated at a temperature of approximately 300° F. at approximately 50 p.s.i.g., the desired drop in pressure being obtained by any suitable means such as a pressure reducing valve (not shown) in line 23. The second fractionator 26 is operated at a temperature of approximately 450° F. at approximately atmospheric pressure to yield a bottoms product having an initial boiling point of approximately 375° F. However where other specialized end products are desired, fractionator 26 may be operated to furnish a bottoms product having an initial boiling point above or below 375° F. as described. The preferred end products are disclosed herein in the sense that such materials show the best balance of physical characteristics, taking vapor pressure, flash point, low temperature, viscosity, and freezing point into account in relation to their effect upon fuel performance in aircraft or missile engines.

The exact reactions which occur in the reactor 21 are not fully understood at present. Primarily, it is believed that alkylation occurs simultaneously or conjointly with dehydrogenation and cyclization. For example, it is probable that hexane in the C<sub>6</sub> reformate becomes dehydrogenated to hexene or benzene which, in turn, acquires ethyl, methyl, or propyl radicals. It may also be that hexene alkylates with other benzene molecules entering via the feed. Similar reactions may occur when iso-octane forms a part of the liquid feed, and similar reactions also may occur where polycyclic compounds are present in or deliberately added to the liquid feed, such as biphenyl. In fact, by addition of biphenyl to the reaction site, such as by introduction thereof into line 15 at a point just ahead of the reactor, the heat content of the end product in terms of B.t.u.'s per gallon may be materially increased, for example, from 128,282 when biphenyl is absent to 132,675 when biphenyl is added to the extent of approximately 10% by weight of the liquid feed component. In place of biphenyl, fused ring aromatic compounds such as naphthalene may be added to the extent of approximately 10% by weight of the liquid feed component. Addition of greater quantities of either of such types of polycyclic aromatic compound is of diminishing advantageousness. Also, as previously noted, while the use of a liquid hydrocarbon feed consisting entirely of C<sub>6</sub> reformate furnishes an end product of high heat content, the heat content of the end product is increased by incorporation of iso-octane or alkylates containing the same. Thus when iso-octane alkylate constitutes 25% by volume of the liquid feed, the heat content is increased approximately 50 B.t.u./lb. over what it would be if this component were omitted from the feed. In general, because of diminishing returns, it appears to be economically undesirable to add alkylate to an extent substantially exceeding 25% by volume of the liquid feed.

The invention has been disclosed particularly in relation to the use of petroleum reformate as the source material for benzene and toluene on account of the economies which the use of reformate provides, but it will be understood that benzene and toluene in admixture produced separately from other petroleum refining methods or from coal tar may be used and that the term "reformate" as used herein is intended to include such alternative source materials.

From the foregoing description of the principles upon which the invention is based and the detailed descriptions of typical procedures, those skilled in the art readily will comprehend the variations to which the invention

is susceptible. By the present process products having unexpectedly high thermal stability characteristics are obtained by mixed reactions conducted simultaneously under mild operating conditions and at low cost of operation. The yield of the desired high performance hydrocarbon end products is not only good but in turn is accompanied by the production of by-products which are adapted to be recycled or sold at favorable prices for other purposes.

Having described my invention, I claim:

1. A process for producing a substantially pure high boiling alkyl naphthenic fuel for use in jet aircraft and missile propulsion which fuel is characterized by an energy content in excess of 18,400 B.t.u. per pound, thermal stability, and resistance to gamma radiation, said process comprising, reacting petroleum reformate and light olefinic hydrocarbons in the range of ethylene, propylene and butylene in admixture with a source of hydroxyl groups, said source being selected from the class consisting of water and alcohol, and hydrogen at a temperature of approximately 150-450° F. in the presence of a phosphoric acid catalyst and at a space velocity in the range of about 0.05 to 1.0 to produce an intermediate product containing highly alkylated benzene compounds, fractionating a high boiling portion of said intermediate product which portion primarily comprises alkyl benzene compounds boiling above about 375° F. and below about 600° F., and hydrogenating said high boiling portion.
2. A process in accordance with claim 1 in which said reformate has an initial boiling point above approximately 140° F. and an end boiling point below approximately 450° F.
3. A process in accordance with claim 1 in which said reformate boils in the range of approximately 250-450° F.
4. A process in accordance with claim 1 in which a minor portion of polycyclic hydrocarbons are added to said reformate and are reacted with said light olefinic hydrocarbons in the presence of said catalyst.
5. A process in accordance with claim 1 in which followinging said hydrogenation, said high boiling portion is contacted with clay at a temperature of about 300-350° F. to effect the polymerization of unstable compounds therein, and in which the polymerized compounds are then filtered from said high boiling portion.
6. A process in accordance with claim 1 in which following said hydrogenation, said high boiling portion is treated with hot clay at a temperature of approximately 300-350° F. and then with cold clay to effect polymerization and removal of unstable hydrocarbons therefrom.
7. A process in accordance with claim 1 in which a fraction of said intermediate product boiling below said high boiling portion is recycled into contact with said catalyst to effect conversion of at least a portion of the recycled fraction into high boiling highly alkylated benzene compounds.
8. A process for producing a substantially pure high boiling naphthenic fuel for use in jet aircraft and missile propulsion which fuel is characterized by an energy content in excess of 18,400 B.t.u. per pound, thermal stability, and resistance to gamma radiation, said process comprising, reacting petroleum reformate and light olefinic hydrocarbon in the range of ethylene, propylene and butylene in admixture with a source of hydroxyl groups, said source being selected from the class consisting of water and alcohol, and hydrogen in the presence of a phosphoric acid catalyst at a space velocity in the range of about 0.05 to 1.0 and at a temperature of approximately 150-450° F. to produce an intermediate product containing highly alkylated benzene compounds, fractionating a high boiling portion of said intermediate product having an initial boiling point above about 375° F. and an end boiling point below about 600° F. and which comprises substantially pure high boiling alkyl benzenes, adding a fused ring compound to said high boiling portion, and hydrogenating the resultant mixture.

9. A process in accordance with claim 8 in which said fused ring compound comprises naphthalene.

10. A process for producing a substantially pure high boiling alkyl naphthenic fuel for use in jet aircraft and missile propulsion which fuel is characterized by its high energy content, thermal stability, and resistance to gamma radiation, said process comprising, contacting admixed petroleum reformate boiling in the range of approximately 140-250° F. and light olefinic hydrocarbons in the range of ethylene, propylene and butylene with a phosphoric acid catalyst at a temperature of approximately 300-400° F., a pressure of approximately 200-400 p.s.i.g., and a space velocity of approximately 0.1 in the presence of water and hydrogen to produce an intermediate product containing alkyl benzene compounds, fractionating a portion of said intermediate product boiling in the range of approximately 375-600° F. and comprising substantially pure alkyl benzenes, and hydrogenating said portion. 15

References Cited in the file of this patent

UNITED STATES PATENTS

|           |                    |       |               |
|-----------|--------------------|-------|---------------|
| 2,202,401 | Rosen              | ----- | May 28, 1940  |
| 2,287,931 | Corson et al.      | ----- | June 30, 1942 |
| 2,335,684 | Mayer              | ----- | Nov. 30, 1943 |
| 2,684,325 | Deanesley          | ----- | July 20, 1954 |
| 2,731,506 | Love et al.        | ----- | Jan. 17, 1956 |
| 2,765,617 | Gluesenkamp et al. | ----- | Oct. 9, 1956  |
| 2,772,215 | Hemminger          | ----- | Nov. 27, 1956 |
| 2,777,007 | Skinner et al.     | ----- | Jan. 8, 1957  |
| 2,910,426 | Gluesenkamp et al. | ----- | Oct. 27, 1959 |
| 2,916,446 | Schuman            | ----- | Dec. 8, 1959  |
| 2,939,833 | Wankat et al.      | ----- | June 7, 1960  |

FOREIGN PATENTS

|         |        |       |              |
|---------|--------|-------|--------------|
| 514,394 | Canada | ----- | July 5, 1955 |
|---------|--------|-------|--------------|

UNITED STATES PATENT OFFICE  
CERTIFICATE OF CORRECTION

Patent No. 3,067,126

December 4, 1962

Arnold M. Leas

It is hereby certified that error appears in the above numbered patent requiring correction and that the said Letters Patent should read as corrected below.

In the grant, lines 1 to 3, for "Arnold M. Leas, of Ashland, Kentucky," read -- Arnold M. Leas, of Ashland, Kentucky, assignor to Ashland Oil & Refining Company, of Ashland, Kentucky, a corporation of Kentucky, --; line 12, for "Arnold M. Leas, his heirs" read -- Ashland Oil & Refining Company, its successors --; in the heading to the printed specification, lines 5 and 6, for "Arnold M. Leas, 803 Bellefonte Princess Road, Ashland, Ky." read -- Arnold M. Leas, Ashland, Ky., assignor to Ashland Oil & Refining Company, Ashland, Ky., a corporation of Kentucky --; column 10, lines 60 and 61, for "hydrocarbon" read -- hydrocarbons --.

Signed and sealed this 11th day of June 1963.

(SEAL)

Attest:

ERNEST W. SWIDER

Attesting Officer

DAVID L. LADD  
Commissioner of Patents